

July 16, 1929.

H. M. NAUGLE ET AL

1,721,351

## CONTINUOUS ANNEALING AND CLEANING PROCESS

Filed Nov. 17, 1924

2 Sheets-Sheet 1



*H.M. Naugle and  
A.J. Townsend*

Frease and Boyd Attorneys

July 16, 1929.

H. M. NAUGLE ET AL

1,721,351

## CONTINUOUS ANNEALING AND CLEANING PROCESS

Filed Nov. 17, 1924

2 Sheets-Sheet 2



Patented July 16, 1929.

1,721,351

## UNITED STATES PATENT OFFICE.

HARRY M. NAUGLE AND ARTHUR J. TOWNSEND, OF CANTON, OHIO, ASSIGNEES; BY MESNE ASSIGNMENTS, TO THE AMERICAN ROLLING MILL COMPANY, OF MIDDLE TOWN, OHIO, A CORPORATION OF OHIO.

### CONTINUOUS ANNEALING AND CLEANING PROCESS.

Application filed November 17, 1924. Serial No. 750,270.

The invention relates to a continuous method for quickly annealing a strip of sheet metal, referred to in a general way in our application for method of making strip sheets filed August 22, 1922, Serial Number 583,612; matured in Patent No. 1,536,028, dated April 28, 1925, and reissued June 14, 1927, Reissue No. 16,652; and the general object of the improvement is to anneal the metal in a manner that will give the product the uniform ductile and other structural characteristics which are necessary for deep drawing and forming or stamping operations.

A readjustment of the grains of the metal to relieve them of the strains produced by a rolling operation, and more particularly by a rapid cold rolling reduction, cannot be accomplished by the ordinary box annealing of a mass or coil of metal, for the reason that the longer period of time required for properly heating the inner portions of the mass or coil, not only results in the overannealing of the outer portion thereof, but in the production of a grain growth in a considerable portion of the mass or coil, which destroys the ductility and uniformity, and also decreases the strength of the material in the outer portions of the mass or coil.

The present improvement is particularly concerned with the annealing of steel having a carbon content of less than .20%, for the reason that such a low carbon steel is best suited for deep drawing and forming or stamping operations; and for properly annealing the same, the metal must be uniformly heated to a temperature of from 1300° to 1600° F. As a grain growth, sometimes known as "Stead's brittleness", may occur at a temperature less than 1400° F., if the same is maintained long enough; one object of the present improvement is to uniformly heat the metal to an annealing temperature, to maintain or continue that temperature only long enough, say from one to three minutes, to correct the micro-structure of the steel which has been critically stressed by previous rolling processes, and then to quickly cool the metal uniformly and gradually, without, however, quenching the same to harden its structure.

The general object of the improvement

may be attained by annealing the strip by the direct action of electric resistors, while moving continuously through a heating chamber, in which the resistors are transversely located adjacent to and parallel with the strip, by which the same may be uniformly heated and the degree of heat definitely controlled at all points in the heating furnace; and then to promptly cool the strip by moving it continuously through a tubular duct surrounded by a moving body of water or other heat absorbing liquid, by which the strip may be quickly and gradually reduced to a non-oxidizing temperature when exposed to the air.

The particular object of the present improvement is to avoid or overcome difficulties which may accompany the continuous annealing processes set forth in our application for patent, filed April 4, 1924, Serial No. 704,157, and the use of the continuous annealing apparatus set forth in our application for patent filed herewith, Serial Number 750,269; in both of which an effort is made to carry on the heating and cooling operations in the presence of a neutral or a reducing gas to the exclusion of air, for preventing or removing an oxidation or discoloration of the surface of the strip.

The very desirable and highly efficient use of electric resistors for directly heating a strip of steel or the like for annealing the same in a chamber containing a reducing gas, requires the use of a refractory lining for the annealing chamber and preferably requires the use of a liquid seal for the opening through which the strip enters the chamber. It has been found, however, that the use of a deoxidizing medium in the heating chamber has an injurious effect upon the electric resistors, and the vapors resulting from the volatilization of a liquid sealing medium has a deteriorating effect upon the refractory lining.

The present improvement avoids these difficulties by the use of an unsealed heating chamber, in which some atmospheric gas may slightly oxidize or discolor the surface of the strip; and by interposing between the heating chamber and the cooling duct of the annealing apparatus, a heat retaining deoxidizing duct containing a reducing gas

for removing any oxidation or discoloration there may be on the strip when it leaves the heating chamber, while in the heated condition.

5 By these means, the detrimental effect upon the refractory lining of the heating chamber by the vapors resulting from volatilization therein of a liquid sealing medium, and the damaging action of a reducing gas 10 upon the electric resistors within the heating chamber, are both avoided; and the heated strip is completely cleaned of any discoloration or oxidation which may be present on its surface, before it enters the cooling 15 duct.

The improved method may be carried out by the apparatus illustrated, more or less continuously, in the accompanying drawings forming part hereof, in which—

20 Figure 1 is a side elevation, partly in section, of the improved apparatus, showing an asbestos seal between the heating and oxidizing ducts;

25 Fig. 2, an enlarged longitudinal section of an asbestos seal;

Fig. 3, is a cross section through the de-oxidizing duct as on line 3—3, Fig. 1; and

30 Fig. 4, a fragmentary side elevation, partly in section showing a liquid seal between the heating and deoxidizing ducts.

Similar numerals refer to similar parts throughout the drawings.

The apparatus may include a coil box A, a strip leveler B, a traveling spot welder 35 C, a solution washer D, an electric heating furnace E, an asbestos seal F, a deoxidizing duct G, a cooling duct H, an exit seal I, conveyer rolls J, a double end shear K, and a strip coiler L, all arranged in series 40 as shown in Fig. 1.

The coil box A may be of any ordinary construction for holding a coil 10 of a strip 11 of steel or the like, and permitting the same to unwind for a continuous annealing; and the strip leveler B may include two sets of rolls 12 of any well known construction and operation, for flattening the sheet and removing uneven fullness or buckles which may have been caused by reducing 45 rolls or other apparatus used in producing the strip.

The spot welder C may include a set of electrodes 13 mounted in a frame 14 supported on a carriage 14' provided with 50 wheels 15 riding on a track 16, together with gripping devices 14" on the front and rear sides of the frame, for clamping and holding successive strips with their ends overlapped, in position between the electrodes 60 for a spot welding operation while the carriage is traveling forward on the track.

The solution washer D may include strip supporting rolls 17 and transverse tubes 18 65 suitably apertured for spraying a hot soda solution upon the strip, to remove grease

and grit therefrom, and like tubes 18' may also be provided for air drying the strip in rear of the cleaner.

The heating furnace E may include a cylindric shell 20 mounted on supports 21 lined with a thick body of heat insulating material 22, within which is provided a lining of fire brick 23 or other refractory material forming a support for electric resistors 24 and 24' parallelly positioned above and below and forming between them a longitudinal heating chamber 25, in which are provided a series of transverse skids 26 for supporting a strip 11 as it is moved endwise through the furnace from the entering slot 20' at its front end to the asbestos seal F at its rear end.

By these means, the strip may be heated directly by the action of the electric resistors, in a uniform manner from end to end of the furnace, and the degree and continuity of heat can be readily controlled at all points in the heating chamber, by referring to the series of pyrometers 25'.

The asbestos seal F may include a box 27 with slots 27' in each end for freely passing a strip sheet 11; above and below which the box is filled with fibrous asbestos 28, supported below by a bottom plate 29 pressed upward by springs 30 and compressed from above by weight plates 31, so as to form a seal by pressing the asbestos against a strip as it is drawn through a box.

The sealing box 27 may be connected to the rear end of the annealing furnace by a flanged funnel nipple 32 and to the front end of the oxidizing duct by a flanged tubular nipple 31'; which nipples are preferably surrounded by an asbestos packing 32' and 32" for retaining the heat.

A water seal F<sup>a</sup> as shown in Fig. 4 may be used in place of the asbestos seal F, and when used, the strip 11 may be guided through the water seal by means of guide rolls f and f' in well known manner.

The deoxidizing duct G may be formed by a metal chamber 33 and a cover 33' mounted on transverse I-bars 34 in a trough channel 35, within which the duct is entirely surrounded with an asbestos packing 36 for retaining the heat within the duct; the chamber being provided with an inlet pipe 33<sup>a</sup> and an outlet pipe 33<sup>a'</sup> for passing a deoxidizing gas through the chamber.

The cooling duct H may be a series of end connected iron tubes 27<sup>a</sup> and 27<sup>a'</sup> extending rearward from the rear end of the furnace, and the sections of the same may be surrounded by tanks or troughs 28 containing water for cooling the conduit and the strip moving through the same.

The cooling troughs may be provided with a water inlet pipe 29<sup>a</sup>, a water connecting pipe 29<sup>a'</sup> and an over-flow pipe 29<sup>a''</sup> so as to cause a continuous flow of cooling

water from the forward toward the rear end of each trough.

The exit seal I may be of the liquid type provided with guide rolls 36' and 36''; and 5 may be provided with an inlet pipe for supplying the same with sealing water or other liquid 37.

The conveyer rolls J may include two 10 strands of pinch rolls 38 arranged for drawing a strip through the apparatus and conveying it rearward to the double shear K, and between these rolls may be provided transverse pipes 31" suitably apertured for hot air drying the strip.

15 The shear K is provided with a shearing die 39 on its front and rear sides and a shearing punch 40 operating between them, for shearing the joint of two strips in front and in rear of their overlapped ends, so as 20 to neatly disconnect them after the annealing process is completed.

25 The strip coiler L may be of any well known construction for winding the annealed strip 11' into a coil 10', and it is preferably provided with an independent motor 34 for this purpose.

30 In the operation of the apparatus, a strip sheet, which has been flattened by the leveler B, joined to another strip by spot welder C, and acted upon by the solution washer D is moved continuously endwise through the heating chamber 25, the deoxidizing duct G, and the cooling duct H; wherein it is heated rapidly and uniformly by the electric resistors to an annealing temperature, which temperature is maintained and continued only 35 for the brief period necessary for a proper annealing of the metal, which may not exceed one minute, whereupon it is deoxidized in the duct G and then promptly cooled gradually by the heat absorbing water surrounding the tubular duct.

40 In this manner a continuous quick annealing and cleaning is accomplished, and 45 the comparatively brief period during which the annealing temperature is maintained and continued, prevents the production of an objectionable grain growth or "Stead's brittleness," so that the annealed strip thus produced is characterized by a uniformly fine 50

grained structure and a highly ductile quality, which adapt it for deep drawing operations.

By the improved apparatus strip sheets of different gauges and of more than ordinary widths can be continuously annealed without developing any objectionable grain growth. 55 In actual practice any given portion of a strip sheet, one-sixteenth of an inch in thickness may be heated to a temperature of 60 1600° F., maintained at that temperature for about one minute, and then cooled to a non-oxidizing temperature, all within a period of about three minutes. This operation can be carried on continuously with respect to all 65 portions of each strip, and of successive strips which have been joined together, without stopping the movement of the strip which is passing through the heating chamber, the deoxidizing duct, and the cooling 70 duct.

Reference is made to our applications for patent filed November 17, 1924, Serial Number 750,271 and the continuation thereof filed July 1, 1925, Serial Number 40,739, containing 75 claims for subject matter disclosed but not claimed therein.

We claim:—

1. The method of annealing the body and cleaning the surface of a steel strip which 80 includes uniformly heating the strip to an annealing temperature, then deoxidizing the surface of the strip while in the heated condition, and then cooling the body thereof, all during a continuous endwise movement 85 of the strip.

2. The method of annealing the body and cleaning the surface of a steel strip which includes uniformly heating the strip to an annealing temperature in an atmospheric gas, 90 and then deoxidizing the surface of the strip while in the heated condition, and subsequently cooling the body thereof in a reducing gas, all during a continuous endwise movement of the strip. 95

In testimony that we claim the above, we have hereunto subscribed our names.

HARRY M. NAUGLE.  
ARTHUR J. TOWNSEND.